

April 3, 1928.

1,664,866

W. O. STODDARD, JR

COATED FABRIC AND PROCESS OF MAKING SAME

Original Filed May 3, 1920

*Fig.I.*



*Fig.II.*



*Fig.III*

*Inventor:*  
William O. Stoddard, Jr.,  
Chester H. Braselton  
*By* C. B. Desjardins  
*Attorneys*

## UNITED STATES PATENT OFFICE.

WILLIAM O. STODDARD, JR., OF DETROIT, MICHIGAN, ASSIGNOR TO DURATEX CORPORATION, OF NEWARK, NEW JERSEY, A CORPORATION OF NEW JERSEY.

## COATED FABRIC AND PROCESS OF MAKING SAME.

Application filed May 3, 1920, Serial No. 378,403. Renewed January 18, 1926.

This invention relates to improvements in coated fabrics and the process of making same. My invention relates more particularly to coated fabrics of the type which are 5 finished or embossed so as to simulate the effect obtained on natural leather.

When natural leather is used in the manufacture of bags, flexible book covers and similar articles, the edge portions of the 10 leather are shaved down to a thin edge. This thin edge is turned upon itself and pasted or otherwise fastened so as to produce a smooth finished binding for the seams of the bag or the edge of the book.

15 This process of shaving down the leather to a thin edge is called skiving and originally it was done with a very sharp shoe-knife. However, at the present time, it is done with a skiving machine. Many attempts have 20 heretofore been made to produce a coated fabric of the type known in the trade as artificial leather which could be subjected to this skiving operation so that hand bags and flexible book covers and similar articles 25 could be made from it having smooth finished seams, produced by the turning over of the skived edges of the coated fabric. So far as I am aware, all of these prior attempts have been unsatisfactory and unsuc- 30 cessful. The reason for this is that the skiving operation would cut the threads of the cloth backing of the artificial leather so that the skived portion of the coated fabric had no tensile strength and would not stand the 35 operation of turning. It will be understood that practically all artificial leather has been produced by applying to a suitable cloth backing, a coating, which is usually composed of a pyroxylin composition carrying 40 the proper pigments or dyes to give the desired color. In the skiving operation the threads of the cloth backing were broken and destroyed so that the pyroxylin film left at the skived edges had no tensile 45 strength.

One of the chief objects of my invention is to produce a coated fabric which may be finished and embossed so as to simulate real leather and which may be skived and 50 turned, as in the case of natural leather, for use in the production of hand bags, flexible book covers and similar articles.

When an artificial leather produced by 55 coating a fabric base with a pyroxylin or nitro-cellulose composition is exposed for

some time to the sun, heat or the effects of weather, it has been found that minute cracks develop in the surface coating which, in time, will permit water to percolate through these cracks so that a coated fabric thus produced is not permanently water proof. It is an object of my invention to provide a coated fabric having a surface coating of pyroxylin or nitro-cellulose which is, nevertheless, permanently water proof 65 and in which means are provided to prevent the percolation of water through the material as a result of the minute cracks appearing in the pyroxylin coating due to exposure to sun, heat and weather. 70

Further objects, and objects relating to details of construction and economies of operation, will more definitely appear from the detailed description to follow. I accomplish the objects of my invention as described in the following specification. My invention is clearly defined in the appended claims. A preferred embodiment of my invention is illustrated in the accompanying drawing, forming a part of this specification, in which 75

Fig. I is a conventional, cross-section view through a piece of coated fabric produced in accordance with my invention;

Fig. II is a similar view showing one edge 80 of the coated fabric skived, preparatory to turning; and

Fig. III is a similar view showing the skived edge turned over upon itself to form the seam. 85

In general, I carry out the objects of my invention by providing a double-texture coated fabric which is made up of two pieces of fabric united together by any suitable adhesive, as by rubber cement, the uppermost 90 fabric having applied thereto a coating of pyroxylin composition which is colored and grained or embossed so as to simulate real leather. In the skiving operation, the lowermost fabric and the cement between the two 95 fabrics is cut away but the cutting does not go far enough to cut the threads of the uppermost fabric which re-inforce the pyroxylin film so that this film has sufficient tensile strength to withstand the operation 100 of turning to form a finished edge as I have described above.

In producing coated fabrics in accordance with my invention, I first take a suitable 105 backing fabric such as a drill, sateen or 110

moleskin and cement to this a thin sheeting which may be of closely woven material. I have secured very satisfactory results by using a rubber cement to join this backing 5 to the thin sheeting which forms a re-inforcing fabric as will appear hereinafter. These two fabrics are joined together by rubber cement on a doubling machine in the manner well-known in the art. It is not necessary 10 to add any description of such a machine at this point because it is well known in the art. After these two fabrics are thus joined together, they are passed into a heater and there vulcanized in the manner well known 15 in the rubber art. I then apply to the light, closely woven sheeting forming the film-reinforcing fabric one or more coatings of a pyroxylin solution to which a vegetable oil and pigment has been added as may be needed. 20 These coatings are applied on a spreading machine by drawing the fabric beneath a spreading knife in the manner well-known in this art. After the application of each coating of the pyroxylin solution, the coated 25 fabric is subjected to a drying operation which evaporates the solvent of the pyroxylin leaving a coating of pyroxylin, vegetable oil and pigment upon the fabric. After the required number of coatings have been applied 30 to the fabric, it is finished by graining or embossing in the manner which is well known in the artificial leather art. It will be understood that the body of the material is made up of the double texture fabric, comprising 35 the two sheets of fabric united by rubber cement and it is only necessary for me to apply a pyroxylin coating of sufficient thickness to enable it to take the graining and embossing operation and to give the finish 40 which is desired.

I have found that it is desirable to use as the top fabric, or the film-reinforcing fabric, a very thin light weight sheeting of fine close weave so that it prevents the pyroxylin solvent from striking through and acting on 45 the rubber cement. I have also found that it is desirable to eliminate, in so far as possible, all ingredients from the pyroxylin coating which might act upon the rubber cement. For instance, benzol is a solvent of rubber 50 and should not be used in the pyroxylin coating in such excess as to strike through into the rubber cement.

I have found that a coated fabric, produced 55 in the manner described above, may be skived in the same manner and with the same results as natural leather. The skiving operation cuts through the backing and rubber cement, but does not cut the threads 60 of the film-reinforcing fabric, so that the skived portion presents a film of pyroxylin which is reinforced by the threads of this top fabric and may be turned upon itself so as to produce the desired results in connection 65 with its use in bookbinding and the

manufacture of ladies' bags, and in similar relations.

I have also found that a coated fabric constructed in accordance with my present invention will be permanently water proof, 70 even though the surface coating of pyroxylin composition be exposed for a long time to the sun, heat or weather. I have found that the intermediate rubber layer by which the two fabrics are joined together, constitutes a 75 water proof layer which will prevent water or moisture from percolating through the material by reason of any minute cracks which may have developed in the surface coating of pyroxylin, due to exposure to sun 80 or heat.

I am aware that the particular embodiment of my invention, which I have described, is susceptible of considerable variation without departing from the spirit 85 thereof and, therefore, I desire to claim the same broadly, as well as specifically, as indicated in the appended claims.

Having thus described my invention, what I claim as new and desire to secure by Letters Patent is:

1. A coated fabric which comprises a fabric base, a relatively thin closely woven top fabric, an intermediate cementing layer of flexible rubber composition uniting said fabric base and said top fabric and a pyroxylin coating covering and supported on said top fabric.

2. A coated fabric which comprises a base fabric, a cementing layer of rubber composition applied to and supported on said base fabric, a surface coating of pyroxylin covering said layer and a fabric separating said surface coating from said rubber layer.

3. A coated fabric comprising a backing 105 composed of two fabrics joined together by a layer of rubber composition interposed between them and vulcanized, one of said fabrics being of relatively close weave, and a surface coating applied to the closely woven 110 fabric separated by said fabric from said rubber layer.

4. A coated fabric composed of a backing comprising two fabrics joined together by a layer of rubber composition interposed 115 between them and vulcanized, one of said fabrics being of relatively light weight and close weave, and a surface coating applied to the closely woven fabric.

5. A coated fabric comprising a backing 120 composed of two fabrics joined together by a layer of rubber composition interposed between them and vulcanized, one of said fabrics being of relatively close weave, and a surface coating of pyroxylin applied to said 125 closely woven fabric.

6. A coated fabric comprising a backing composed of two fabrics joined together by a layer of rubber composition interposed 130 between them and vulcanized, one of said

fabrics being of relatively light weight and close weave, and a surface coating of pyroxylin applied to said closely woven fabric.

7. A coated fabric composed of a backing comprising two fabrics joined together by a layer of rubber composition interposed between them and vulcanized, one of said fabrics being of relatively close weave, and a surface coating of pyroxylin applied to and supported on the close woven fabric separate from the underlying layer of rubber composition, whereby said coated fabric may be subjected to a skiving operation without destroying the tensile strength of said surface coating.

8. The process of making coated fabrics comprising joining two fabrics together by a layer of rubber cement interposed between them, and applying a pyroxylin surface coating to one of said fabrics while avoiding a commingling of said cement layer and said surface coating.

9. The process of making coated fabrics comprising joining two fabrics together by a layer of rubber cement, vulcanizing said material, and then applying a surface coating to one of said fabrics while preventing said surface coating from uniting directly with said layer of rubber cement.

10. The process of making coated fabrics comprising joining two fabrics together by a layer of rubber cement interposed between them, one of said fabrics being of relatively close weave, and then applying a surface coating of pyroxylin composition having a benzol content so low as not to act appreciably on the rubber layer, to the closely woven fabric.

11. The process of making coated fabrics comprising joining together two fabrics by a layer of rubber composition interposed between them, one of said fabrics being of relatively close weave and light weight, vulcanizing the material thus formed, and then applying a surface coating of pyroxylin to the closely woven fabric.

12. The process of making coated fabrics which consists in applying to the surface of a base fabric a layer of rubber cement; superposing on the cement a second fabric; applying a number of coats of pyroxylin solution successively to the second fabric; subjecting each coat to a drying operation; and finally finishing the pyroxylin surface.

In testimony whereof, I affix my signature.

WILLIAM O. STODDARD, JR.